# EUROPEAN PATENT APPLICATION

(11) **EP 4 700 143 A1**
(43) Date of publication of application: **25.02.2026**
(21) Application number: 24792632.2
(22) Date of filing: 15.04.2024
(51) Int. Cl.: C22C 38/00, C21D 6/00, C21D 6/04, C22C 38/10

(54) **LOW THERMAL EXPANSION STEEL CASTING PRODUCT AND METHOD FOR MANUFACTURING SAME**

(30) Priority: 19.04.2023 JP 2023068722
(71) Applicant: Shinhokoku Material Corp., Saitama 350-1124 (JP)
(72) Inventor: OHNO, Haruyasu, Kawagoe-shi, Saitama 350-1124 (JP); ONA, Kotaro, Kawagoe-shi, Saitama 350-1124 (JP)
(74) Representative: Vossius & Partner Patentanwälte Rechtsanwälte mbB
(86) International application number: PCT/JP2024/014980
(87) International publication number: WO 2024/219358

(57) **Abstract**

The present invention addresses the problem of providing a low thermal expansion cast steel product having excellent plating properties. A low thermal expansion cast steel product according to the present invention has a chemical composition containing, in mass%, 0.040% or less of C, 0.30% or less of Si, 0.50% or less of Mn, 0.010% or less of S, 31.00-34.00% of Ni, 4.90-6.00% of Co, 0.0100% or less of O, and 0.010-0.100% of Al, the remaining portion being Fe and unavoidable impurities, has an austenite structure having an average grain size of 200 µm or less, and has an average thermal expansion coefficient of 0.4×10^{- 6} /°C or less at 25-100°C.

## Description

### FIELD

The present invention relates to a low thermal expansion cast steel product having a low coefficient of thermal expansion and a method for producing the same.

### BACKGROUND

Thermally stable Invar alloy is widely used as component materials for electronics, semiconductor-related equipment, laser processing machines, and ultra-precision processing equipment.

PLT 1 discloses a low thermal expansion alloy having a coefficient of thermal expansion of 0.5×10⁻⁶/°C to 2.0×10⁻⁶/°C, which comprises Ni: 29.5 to 35%, Co: 2.0 to 7.0%, Cr: 0.001 to 2.0 %. This alloy is obtained by after homogenous solution treatment process, quenching or annealing with cooling rate of 1°C/sec or less, and performing cold rolling of 10% or more.

PLT 2 discloses a low thermal expansion line comprising Co: 65% or less, Ni: 30% or less and Cr: 10% or less, wherein a total content of Co and Ni is 25 to 65%. PLT 2 discloses a method of transforming a part of an austenite phase of a low thermal expansion line into a deformation-induced martensite phase of by cold working.

PLT 3 discloses a low thermal expansion alloy comprising Ni: 0.03 to 1.5%, total of Ni and Co: 53 to 55%, and Cr: 9 to 10%. PLT 3 discloses a method comprising annealing the alloy at 650 to 900°C and then cooling at a rate of less than 20°C/min in a furnace.

### [CITATIONS LIST]

### [PATENT LITERATURE]

[PLT1] JP 2796966 B
[PLT2] JP H 6-279945 A
[PLT3] JP 5534150

### SUMMARY

### [TECHNICAL PROBLEM]

When the low thermal expansion cast steel is plated, a pretreatment is performed. In the pretreatment, etching is performed, and in this case, an etch pit may occur on the surface of the steel casting product. If the etch pit is formed, the plating property is deteriorated, and a pinhole may be formed when plating.

The object of the present invention is to solve the above-mentioned problems and to provide a low thermal expansion cast steel product having good plating properties, in which occurrence of etch pits in a pretreatment of plating is suppressed.

### [SOLUTION TO PROBLEM]

The present inventors have intensively studied a method of suppressing an etch pit in a low thermal expansion cast steel product, and have made the present invention. The present invention includes the following embodiments.
(1) A low thermal expansion cast steel product, having a chemical composition comprising, by mass%, C: 0.040% or less, Si: 0.30% or less, Mn:0.50% or less, S: 0.010% or less, Ni: 31.00 to 34.00%, Co: 4.90 to 6.00%, O: 0.0100% or less, Al: 0.010 to 0.100%, and balance of Fe and unavoidable impurities, having average crystal grain size of an austenite structure of 200µm or less, having a mean coefficient of thermal expansion in 25 to 100°C of 0.4× 10^{- 6} /°C or less.
(2) A method of manufacturing the low thermal expansion cast steel product according to claim 1, the method comprising, in order, a cryogenic treatment step of cooling a steel casting product having a chemical composition comprising, by mass%, C: 0.040% or less, Si: 0.30% or less, Mn:0.50% or less, S: 0.010% or less, Ni: 31.00 to 34.00%, Co: 4.90 to 6.00%, O: 0.0100% or less, Al: 0.010 to 0.100%, and balance of Fe and unavoidable impurities, to Ms point or less, holding the steel casting product for 0.5 to 3hr at a temperature of Ms point or less, and heating the steel casting product to room temperature; and a recrystallization step of heating the steel casting product to 800 to 1100°C, holding the steel casting product for 0.5 to 5hr, and quenching.

### [ADVANTAGEOUS EFFECTS OF INVENTION]

According to the present invention, it is possible to obtain a low thermal expansion cast steel product having good plating property.

### BRIEF DESCRIPTION OF DRAWINGS

[Fig. 1] Fig. 1 shows an example of the structure of the steel casting product after cryogenic treatment.
[Fig. 2] Fig. 2 shows an example of the structure of the steel casting product after recrystallization.

### DESCRIPTION OF EMBODIMENT

Hereinafter, the present invention will be described in detail.

### <Chemical composition>

First, the chemical composition of the steel casting product of the present invention will be described. Hereinafter, "%" with respect to the chemical composition represents "mass%" unless otherwise specified.

### (C: 0.040% or less)

C is a solid solution in austenite contributes to increase in strength. However, C is dissolved in the matrix in the recrystallization step, precipitates during cooling, and increases the coefficient of thermal expansion. In order to reduce the coefficient of thermal expansion at 25 to 100°C to 0.4 10⁻⁶/°C or less, the amount of the deposition of C must be reduced. Therefore, the content of C is 0.040% or less. The content of C may be 0.035% or less, 0.030% or less, 0.025% or less, or 0.020% or less. The content of C may be 0.001% or more, 0.002% or more, 0.003% or more, 0.004% or more, or 0.005% or more.

### (Si: 0.30% or less, Mn: 0.50% or less)

Si and Mn are added as deoxidizers. In the present invention, in order to produce a good steel casting product without blowing, it is sufficient to add the minimum amount necessary for deoxidation, respectively. The steel casting product to be finally produced does not need to contain Si and Mn, and the content of Si and the content of Mn may be 0%. However, Si may be contained in 0.30 % or less and Mn may be contained in 0.50 % or less, respectively. Since deoxidation can also be carried out by Al, Si and Mn may not be added. The content of Si may be 0.25% or less, 0.20% or less, 0.15% or less, or 0.10% or less. The content of Si may be 0.01% or more, 0.02% or more, 0.03% or more, 0.04% or more, or 0.05% or more. The content of Mn may be 0.40% or less, 0.30% or less, or 0.20% or less. The content of Mn may be 0.01% or more, 0.05% or more, 0.08% or more, 0.10% or more, 0.12% or more, or 0.15% or more.

### (S: 0.010% or less)

S is contained as an impurity. S produces sulfide, and the generated sulfide causes the generation of etch pits during the pretreatment of plating. In order to suppress the generation of sulfides, the content of S is set to 0.010% or less. The content of S may be 0.009% or less, 0.008% or less, 0.007% or less, 0.006% or less, or 0.005% or less. The smaller the S content, the better. Therefore, the content of S may be 0%. However, since setting the content of S to 0% would increase costs, the content of S may be 0.001% or more, or 0.002% or more.

### (Ni: 31.00 to 34.00%)

Ni is an element which reduces the coefficient of thermal expansion. If the content of Ni is too large or too small, the thermal expansion coefficient is not sufficiently low. Further, if the content of Ni is too large, it becomes difficult to cause martensitic transformation by cooling. The content of Ni must be controlled to a narrow range in order to reduce the coefficient of the thermal expansion at 25 to 100°C to 0.4 × 10⁻⁶/°. In particular, the content of Ni is 31.00 to 34.00%. The content of Ni may be 31.20% or more, 31.30% or more, or 31.50% or more. The content of Ni may be 33.50% or less, 33.00% or less, or 32.50% or less.

### (Co: 4.90 to 6.00%)

Co contributes to decrease in the coefficient of thermal expansion by being combined with Ni. The content of Co must be controlled to a narrow range in order to reduce the coefficient of the thermal expansion at 25 to 100°C to 0.4 × 10⁻⁶/°C. In particular, the content of Co is 4.90 to 6.00%. The content of Co may be 5.80% or less, 5.70% or less, 5.60% or less, 5.50% or less, or 5.40% or less. The content of Co may be 4.95% or more, 5.00% or more, 5.05% or more, 5.10% or more, or 5.15% or more.

### (O: 0.0100% or less)

O is contained as an impurity. O generates an oxide, and the generated oxide causes the generation of etch pits during the pretreatment of plating. In order to suppress the generation of oxides, the content of O should be 0.0100% or less. The content of O may be 0.0090% or less, 0.0080% or less, 0.0070% or less, 0.0060% or less, or 0.0050% or less. The lower the content of O, the better, and the content of O may be 0%. However, since setting the content of O to 0% would increase cost, the content of O may be 0.0001% or more, 0.0005% or more, 0.0010% or more, 0.0015% or more, or 0.0020% or more.

### (Al: 0.010 to 0.100%)

Al is added as a deoxidizer. In the low thermal expansion cast steel of the present invention disclosure, enough amount of Al is contained in order to make the content of O 0.0100% or less. Therefore, the content of Al in the steel casting product to be finally produced should be 0.010 to 0.100%. The content of Al may be 0.015% or more, 0.020% or more, 0.025% or more, 0.030% or more, 0.035% or more, or 0.040% or more. The content of Al may be 0.090% or less, 0.085% or less, 0.080% or less, 0.075% or less, or 0.070% or less.

The balance of the chemical composition is Fe and unavoidable impurities. The unavoidable impurities mean compositions which are not intentionally contained in the steel, but unavoidably mixed, from raw materials, manufacturing environment, and the like, when the steel having the chemical composition specified in the present invention is industrially manufactured. The unavoidable impurities include P, Cu, and the like, which are elements not intentionally added in the manufacturing process. The content of the impurity is not limited as long as it does not affect the effect of the present invention. The content of the impurity may be 0.50% or less, 0.40% or less, 0.30% or less, 0.20% or less, 0.15% or less, 0.10% or less, 0.05% or less, or 0% by mass in total.

### <Microstructure of steel casting product>

The microstructure of the steel casting product of the present invention is an austenitie structure having an average grain size of 200µm or less. The structure mainly comprises fine equiaxed grain. It is not necessary that all of the structures are equiaxed grains, but it is preferable that the ratio of equiaxed grain is 60% or more in area ratio. The ratio of the equiaxed grain is more preferably 90% or more, and even more preferably 95% or more in area ratio.

The average crystal grain size of austenite was determined as the average value of the circle equivalent diameter of the grains observed under an optical microscope after cutting a sample for microstructural observation from the center of the steel casting product, polishing the observation surface to a mirror finish, and etching it with Marble reagent.

### <Coefficient of thermal expansion>

The steel casting product of the present invention has an coefficient of thermal expansion of 0.4 × 10⁻⁶ at 25 to 100°C or less. The coefficient of thermal expansion is measured as the coefficient of thermal expansion at 25 to 100°C by sampling a thermal expansion measuring test piece from the vicinity of the center of the steel casting product and heating the test piece at a heating rate of 3°C/min from 0°C to 130°C using a thermal expansion measuring device. As the thermal expansion measuring device, it is possible to use a DIL 402C manufactured by NETZSCH. The coefficient of thermal expansion at 25 to 100°C may be 0.40 × 10⁻⁶/°C or less, 0.35 × 10⁻⁶/°C or less, 0.30 × 10⁻⁶/°C or less or 0.25 × 10⁻⁶/°C or less.

### <<Manufacturing method>>

Next, a method of manufacturing the low thermal expansion cast steel product of the present invention will be described.

### (Casting)

First, molten steel prepared so that the steel casting product has the chemical composition described above is produced. The method for producing molten steel is not particularly limited, and a known apparatus and method may be used. Then, the molten steel is poured into a casting mold and solidified to obtain a steel casting product. The casting mold, the pouring device for pouring molten steel into the casting mold, and the pouring method are not particularly limited, and known apparatuses and methods may be used. The microstructure of the steel casting product produced by the casting mold becomes a microstructure mainly comprising the columnar crystal. The obtained steel casting product is subjected to the following heat treatment.

### (Cryogenic treatment step)

Next, the steel casting product is rapidly cooled to a Ms point or lower, and is held at a temperature below Ms point for 0.5 to 3hr, and then the temperature is raised to room temperature (cryogenic treatment step). The method of cooling is not particularly limited. Ms point can be estimated by the following equation using the composition of the steel, generally.

$Ms \left(C ∘\right) = 521 - 353 C - 22 Si - 24.3 Mn - 7.7 Cu - 17.3 Ni - 17.7 Cr - 25.8 Mo$

Here, C, Si, Mn, Cu, Ni, Cr, and Mo are contents (mass%) of the respective elements. For elements which are not contained, 0 is substituted.

For the chemical composition of the low thermal expansion cast steel product of the present invention, Ms point calculated by the above equation, in particular depending on the content of Ni, is about -10°C to -70°C. Therefore, as the cooling method, immersing dry ice and methyl alkol or ethyl alcohol, or liquid nitrogen, or spraying liquid nitrogen may be used. As a result, a microstructure containing fine martensite is generated. Further, rising the temperature may be performed by pulling up to room temperature air. FIG. 1 shows an example of the microstructure after the cryogenic treatment step. In the microstructure photograph, the black portion is martensite. The generation of a large amount of martensite results in a refinement of the austenitic grain size in the subsequent recrystallization step.

### (Recrystallization treatment step)

Next, the steel casting product is reheated to 800 to 1100°C, held at 800 to 1100°C for 0.5 to 5hr, and quenched. As a result, the microstructure in which martensite is generated returns to the austenite structure. Although crystal grain size of the microstructure generated by general solidification is about 1 to 10mm, through the above cryogenic treatment step and subsequent recrystallization step, the austenite structure becomes a fine structure mainly comprising equiaxed grain and having an average grain size of 200µm or less. The cooling rate of the quenching is preferably 10°C/min or more, more preferably 30°C/min or more, and more preferably 100°C/min or more at an average cooling rate from the holding temperature to room temperature. FIG. 2 shows an example of the microstructure after the recrystallization step. It can be confirmed that the microstructure after the recrystallization step is a fine structure having an average grain diameter of 200µm or less.

### (Solution treatment step)

Before the cryogenic treatment, a solution treatment step may be provided in which the steel casting product is heated to 800 to 1100°C, held 0.5 to 5hr, and quenched. The solution treatment step is not an essential step and may be performed as necessary. By solution, the precipitate precipitated during casting is dissolved, and ductility, toughness is improved.

### (Diffusion treatment step)

Before the cryogenic treatment step (before the solution treatment step when the solution treatment step is provided), a diffusion treatment step of holding the steel casting product at 1100 to 1300°C for 5 to 50hr may be further provided. The diffusion treatment step is not an essential step and may be performed as necessary. By this step, segregation of Ni and impurities in the steel is eliminated, and even a steel casting product has a large size, the steel casting product having a low coefficient of thermal expansion can be produced more stably.

### (Tempering treatment step)

Between the cryogenic treatment step and recrystallization step, a martensitic tempering treatment is performed by heating the steel casting product to 300 to 400°C just below AC₃ point and holding it for 1 to 10hr at 300 to 400°C in order to refine the recrystallized austenite grains. The tempering treatment step is not an essential step and may be performed as needed.

### EXAMPLES

### <Inventive Example 1>

Using a high-frequency induction furnace, the molten metal was poured into the casting mold, and a Y-shaped test material having the composition shown in No.1 of Table 1 was produced. The produced Y-type test material was subjected to cryogenic treatment of cooling to -80°C and holding for 1.5hr, then tempering treatment of heating to 350°C and holding for 4hr, further, recrystallization of reheating to 1100°C, holding for 2.0hr, and quenching at a cooling rate of 2000°C/min to obtain a low thermal expansion cast steel product.

### <Inventive Examples 2 to 8 and Comparative Examples 1 to 6>

Low thermal expansion steel casting products were obtained in the same manner as in Example 1 except that the chemical composition, the temperature of the cryogenic treatment, and the temperature of the recrystallization were set to the conditions described in Tables 1 and 2. For each treatment temperature in Table 2, "-" means that the process was not provided. Also, in Inventive Example 6 and Comparative Example 5, the diffusion treatment step described above was provided before the cryogenic treatment step. In Inventive Examples 7 and 8, and Comparative Example 6, the solution treatment step described above was provided before the cryogenic treatment step. In Inventive Example 8, a diffusion treatment step was further provided before the solution treatment step. In Inventive Examples 1, 2, 6, and 8, and Comparative Examples 1, 2, and 4, the above-described tempering treatment step was provided between the cryogenic treatment step and the recrystallization step. The holding temperatures of the diffusion treatment step, the solution treatment step, and the tempering treatment step were as shown in Table 2, and the holding times were 20hr, 2hr, 5hr, respectively. Ms points shown in Table 2 are calculated by the above-described estimation equation.

### (Average crystal grain size of austenite, coefficient of thermal expansion at 25 to 100°C)

For the obtained low thermal expansion cast steel product, the average crystal grain size of austenite and the coefficient of thermal expansion at 25 to 100°C were determined by the above-described method.

### (Plating property)

Plating property was evaluated by the following method. The surface of samples of 50mm×50mm× thickness 10mm from the obtained low thermal expansion cast steel product were pickled with hydrochloric acid, further, pickled with a mixed solution of hydrochloric acid and sulfuric acid, and were immersed for 8 hours so that thickness of Ni plating was about 100µm.

For the sample after plating, 50mm×50mm surface was observed by an optical microscope, was evaluated in the presence of plating defects (pinholes) having a diameter of more than 200µm. When no pinhole was observed, it was determined that the plating property was good.

The above results are shown in Table 2.

### [Table 1]

**Table 1**

| No. | Chemical composition (mass%) balance: Fe and impurities | | | | | | | |
|---|---|---|---|---|---|---|---|---|
| | C | Si | Mn | S | Ni | Co | Al | O |
| Inv. ex. 1 | 0.005 | 0.10 | 0.16 | 0.004 | 31.37 | 5.18 | 0.070 | 0.0032 |
| Inv. ex. 2 | 0.002 | 0.04 | 0.21 | 0.003 | 33.16 | 5.09 | 0.020 | 0.0021 |
| Inv. ex. 3 | 0.017 | 0.09 | 0.18 | 0.003 | 31.98 | 5.21 | 0.045 | 0.0026 |
| Inv. ex. 4 | 0.012 | 0.15 | 0.19 | 0.004 | 32.30 | 5.44 | 0.027 | 0.0031 |
| Inv. ex. 5 | 0.008 | 0.13 | 0.23 | 0.006 | 31.70 | 5.86 | 0.023 | 0.0019 |
| Inv. ex. 6 | 0.005 | 0.10 | 0.16 | 0.004 | 31.37 | 5.18 | 0.070 | 0.0032 |
| Inv. ex. 7 | 0.002 | 0.04 | 0.21 | 0.003 | 33.16 | 5.09 | 0.020 | 0.0021 |
| Inv. ex. 8 | 0.017 | 0.09 | 0.18 | 0.003 | 31.98 | 5.21 | 0.045 | 0.0026 |
| Comp. ex. 1 | 0.002 | 0.04 | 0.17 | 0.003 | 32.75 | 3.46 | 0.052 | 0.0029 |
| Comp. ex. 2 | 0.009 | 0.09 | 0.24 | 0.019 | 32.41 | 6.49 | 0.034 | 0.0450 |
| Comp. ex. 3 | 0.001 | 0.08 | 0.38 | 0.007 | 35.63 | 4.90 | 0.002 | 0.0142 |
| Comp. ex. 4 | 0.006 | 0.36 | 0.62 | 0.008 | 30.40 | 4.50 | 0.013 | 0.0036 |
| Comp. ex. 5 | 0.002 | 0.04 | 0.17 | 0.003 | 32.75 | 3.46 | 0.052 | 0.0029 |
| Comp. ex. 6 | 0.009 | 0.09 | 0.24 | 0.019 | 32.41 | 6.49 | 0.034 | 0.0450 |

| | | | | | | | | |
|---|---|---|---|---|---|---|---|---|
| * Underlines indicate outside scope of present invention. | | | | | | | | |

### [Table 2]

**Table 2**

| No. | Temperature of diffusion treatment | Temperature of solution treatment | MS point | Temperature of cryogenic treatment | Temperature of tempering treatment | Temperature of recrystallization | Crystal grain size | Coefficient of thermal expansion (25 to 100°C) | Plating property (presence or absence of pinhole) |
|---|---|---|---|---|---|---|---|---|---|
| | [°C] | [°C] | [°C] | [°C] | [°C] | [°C] | [µm] | [× 10-⁶/°C] | |
| Inv. ex. 1 | - | - | -30 | -80 | 350 | 1100 | 120 | 0.30 | absence |
| Inv. ex. 2 | - | - | -59 | -196 | 400 | 850 | 95 | 0.34 | absence |
| Inv. ex. 3 | - | - | -45 | -196 | - | 900 | 75 | 0.25 | absence |
| Inv. ex. 4 | - | - | -50 | -196 | - | 900 | 50 | 0.31 | absence |
| Inv. ex. 5 | - | - | -39 | -80 | - | 1000 | 105 | 0.37 | absence |
| Inv. ex. 6 | 1200 | - | -30 | -80 | 300 | 900 | 110 | 0.25 | absence |
| Inv. ex. 7 | - | 900 | -59 | -196 | - | 1000 | 50 | 0.21 | absence |
| Inv. ex. 8 | 1150 | 800 | -45 | -196 | 300 | 850 | 60 | 0.18 | absence |
| Comp. ex. 1 | - | - | -51 | -196 | 320 | 800 | 80 | 0.53 | absence |
| Comp. ex. 2 | - | - | -51 | -196 | 350 | 1000 | 150 | 0.73 | presence |
| Comp. ex. 3 | - | - | -107 | - | - | - | 1200 | 2.78 | presence |
| Comp. ex. 4 | - | - | -30 | -80 | 300 | 1100 | 70 | 2.30 | absence |
| Comp. ex. 5 | 1200 | - | -51 | -196 | - | 900 | 70 | 0.50 | absence |
| Comp. ex. 6 | - | 1000 | -51 | -196 | - | 1100 | 145 | 0.69 | presence |

| | | | | | | | | | |
|---|---|---|---|---|---|---|---|---|---|
| * Underlines indicate outside scope of present invention or desired properties not obtained. | | | | | | | | | |

As shown in Table 2, it was confirmed that the low thermal expansion cast steel products of the invention examples had a low coefficient of thermal expansion at 25 to 100°C and also had good plating properties.

In Comparative Example 1, since the content of Co was small, the coefficient of thermal expansion increased.

In Comparative Example 2, since the contents of Co, S, and O were large, the coefficient of thermal expansion increased, and the plating property was poor.

Comparative Example 3 is an example in which the content of Ni is large, the content of Al and O is small, and further, the cryogenic treatment and the recrystallization are not performed. As a result, the grain size was not refined, the coefficient of thermal expansion increased, and the plating property was poor.

In Comparative Example 4, since the content of Si, Mn was large and the content of Ni and Co was small, the coefficient of thermal expansion increased.

In Comparative Example 5, since the content of Co was small, the coefficient of thermal expansion increased.

In Comparative Example 6, since the contents of Co, S, and O were large, the thermal expansion coefficient increased, and the plating property was poor.

## Claims

1. A low thermal expansion cast steel product,
having a chemical composition comprising, by mass%,
C: 0.040% or less,
Si: 0.30% or less,
Mn:0.50% or less,
S: 0.010% or less,
Ni: 31.00 to 34.00%,
Co: 4.90 to 6.00%,
O: 0.0100% or less,
Al: 0.010 to 0.100%, and
balance of Fe and unavoidable impurities,
having average grain size of an austenite structure of 200µm or less,
having a mean coefficient of thermal expansion in 25 to 100°C of 0.4× 10⁻⁶/°C or less.

2. A method of manufacturing the low thermal expansion cast steel product according to claim 1, the method comprising, in order,
a cryogenic treatment step of cooling a steel casting product having a chemical composition comprising, by mass%,
C: 0.040% or less,
Si: 0.30% or less,
Mn:0.50% or less,
S: 0.010% or less,
Ni: 31.00 to 34.00%,
Co: 4.90 to 6.00%,
O: 0.0100% or less;
Al: 0.010 to 0.100%, and
balance of Fe and unavoidable impurities,
to Ms point or less, holding the steel casting product for 0.5 to 3hr at a temperature of Ms point or less, and heating the steel casting product to room temperature; and
a recrystallization step of heating the steel casting product to 800 to 1100°C, holding the steel casting product for 0.5 to 5hr, and quenching.
